

## UNITED STATES PATENT OFFICE

2,347,178

## REVERSIBLE EMULSION AND APPLICATION THEREFOR

James H. Fritz, Montclair, and Edwin A. Robinson, Chatham, N. J., assignors to National Oil Products Company, Harrison, N. J., a corporation of New Jersey

No Drawing. Application January 7, 1942,  
Serial No. 425,856

15 Claims. (CL 252—312)

This invention relates to emulsions of water-in-oil, oil-in-water and intermediate types, and more particularly to such emulsions which are stabilized by means of cationic surface active amino compounds.

Heretofore emulsions of water in oil have been prepared which are convertible by dilution and vigorous agitation to emulsions of oil in water. However, it has not been possible to prepare emulsions of water in oil which are stable at or near the inversion point or which may be converted by very mild agitation and dilution to oil-in-water emulsions, notwithstanding the considerable need for such stable and readily invertible emulsions.

Accordingly, it is an object of this invention to provide water-in-oil emulsions which can be readily and smoothly inverted and which will be stable at or near the inversion point.

Another object is to provide a water-in-oil emulsion which can be added to a batch or stream of aqueous stock in process to obtain the effect of adding an oil, without, however, encountering any subsequent difficulties due to separation of the oil from the stock.

A further object is to provide an agent and process for defoaming aqueous stock which will require only a minimum quantity of material and which will not interfere with any subsequent operations upon the stock.

The above and other objects are secured by this invention in an emulsion of an oily material, such as a petroleum oil and water, stabilized by a cationic surface active fatty amino compound, such as the amide produced by reacting oleic acid with diethylene triamine, which compound is adjusted by means of a weak acid, such as acetic acid, to a pH of 6 or below. At moderate concentration of the oil, the oil will be the continuous phase, but upon dilution with water the emulsion inverts to become an oil-in-water emulsion. Both the undiluted and diluted emulsions are entirely stable at any point in the process of inversion, which will take place without the separation of any macroscopic phase and with only the slight agitation necessary to secure mixing. The diluted and inverted emulsions are not like other oil-in-water emulsions, but have properties similar to water-in-oil emulsions; for instance, they have a greasy feel and tend to prevent any foaming of solutions into which they are incorporated. These properties suggest the use of these emulsions for many applications, as where it is desired to treat an aqueous stock with an oily material and to have the oily mate-

rial eventually disperse throughout the stock without separating. Specifically, it is often desired to break the foam on the surface of paper stock, glue, starch, casein solutions undergoing enzymatic and hydrolytic processes and the like, by adding an oily material thereto. The emulsions of this invention will act as such an oil, but will eventually disperse smoothly and completely throughout the body of the stock and thus avoid interference with any subsequent operations.

The amide of oleic acid with ethylene diamine was cited as a suitable emulsifying agent for the practice of this invention, but any fatty compound having at one end a fatty residue of 10 or more carbon atoms and no hydrophilic groups, and presenting at the other extremity an amine group, will be suitable. Examples of such compounds are fatty amines and the amides of the fatty acids with the polyamines. As an acid residue in such an amide there may be cited oleic acid, lauric acid, myristic acid, palmitic acid, stearic acid, palmitoleic acid, arachidic acid and the like. Instead of the pure acids the fatty acid residues contained in fats and oils, such as coconut oil, soyabean oil, lard, tallow, peanut oil, corn oil, hydrogenated soyabean oil, hydrogenated fish oil, and the like may be employed. The amide residue may be derived from any polyamine such as ethylene diamine, diethylene triamine, ethanol ethylene diamine, tetraethylene pentamine, 1,3 diamino isopropanol and the like. Specific amides coming within the above requirements are exemplified in the amide produced by reacting oleic acid and ethylene diamine; rice oil with diethylene triamine; soyabean oil with diethylene triamine, hydrogenated soyabean oil with ethanol ethylene diamine, etc. Examples of suitable amines are stearyl amine, oleyl amine, lauryl amine, dilauryl amine, and the like.

Acetic acid was cited as a suitable acid for adjusting the pH of the cationic surface active amino compound. However, any acid may be used for this purpose, preferably a weak acid, in order that the pH may be adjusted more accurately and that a buffering action may be secured. A sufficient amount of the acid is employed to reduce the pH of the amino compound to 6 or below when the amino compound is in 2% aqueous solution.

Petroleum oil was cited as an oil suitable for the oily phase of emulsions according to this invention. However, any mineral, vegetable or animal oil, fat or wax, the viscosity of which is not too great to interfere with the inversion of the

phases, may be employed. Mineral oils may vary in viscosity from about 35 seconds to 300 seconds Saybolt (100° F.). Suitable oils, other than mineral oils, are exemplified in soyabean oil, cottonseed oil, rice oil, peanut oil, corn oil, tea-seed oil, neat's-foot oil, cod oil, castor oil, whale oil, sperm oil, lard oil, sardine oil, and blown or polymerized products produced from these oils.

Emulsions prepared as above described are stable under varying conditions of storage even in the vicinity of the inversion point. The emulsions invert readily by dilution, in most cases with no more agitation than is necessary to secure even distribution of the materials. These properties render the emulsions very advantageous for many uses; for instance, it is possible to ship to the consumer a very concentrated emulsion containing mostly oil, which emulsion may be converted at the point of use into an oil-in-water emulsion without difficulty or special equipment. Further, the diluted and inverted emulsions have the properties unlike those of most oil-in-water emulsions, in that they have a greasy feel and a tendency to prevent and destroy foam on any aqueous bodies containing them. Further, when these emulsions are added to any batch or stream of materials in process, they will exert the same action as an unemulsified oil would, with the advantages that a considerably less amount of actual oil is used, since the bulk of the emulsion will be constituted of water, and further, that the emulsion will subsequently disperse completely in the stock without separating and interfering at subsequent points in the process. For instance, the emulsions may be added to paper or glue stocks at any point where foaming is encountered and will kill the foam at that point. However, the oil will eventually become distributed thoroughly throughout the body of the stock and will not cause troubles such as, in the case of the paper, streaks in the paper web made therefrom, or in the case of glue, fish eyes on the coatings made therefrom. Further, these emulsions will not readily attack the rubber or other oil-sensitive materials contacted by the stock to which they are added.

For a fuller understanding of the nature and objects of the invention, reference should be had to the following examples which are given merely to further illustrate the invention, and are not to be construed in a limiting sense, all parts given being by weight.

#### Example I

270 parts of #2 fuel oil, 30 parts of the monoamide produced by reacting oleic acid with ethylene diamine, and 1 part of glacial acetic acid were mixed. 300 parts of water were added and mixed in with agitation to form an emulsion of water in oil. 200 additional parts of water were stirred in and there resulted an emulsion which apparently contained both oil in water and water in oil phases, but which did not separate any macroscopic phase. 800 additional parts of water were added and there resulted an emulsion in which water was the continuous phase, the inversion taking place smoothly and with only moderate agitation. This emulsion had a greasy feel and could be diluted indefinitely with water without breaking.

An emulsion of water in oil prepared as just described, but without having been diluted with water, was added to a stream of paper stock going to the vat of a cylinder machine, in which foam-

ing was giving trouble. The foam broke down immediately.

#### Example II

5 270 parts of #2 fuel oil, 30 parts of the monoamide produced by the reaction of hydrogenated soyabean oil with ethanol ethylene diamine, and 1 part of glacial acetic acid were mixed. 300 parts of water were added and mixed in with agitation to form an emulsion of water in oil. This emulsion exhibited the same capability of inversion to an oil-in-water emulsion as the emulsion in Example I. The emulsion of this example had excellent defoaming properties.

#### Example III

10 30 parts of the monoamides formed by reacting a mixture of rice oil and cottonseed oil with diethylene triamine were substituted for the monoamides employed in the procedures of Examples I and II. The resulting water-in-oil emulsions exhibited the same properties of ready inversion and of foam prevention as did the emulsions in Examples I and II.

#### Example IV

15 20 25 The procedures of Examples I and II were repeated, using stearylamine in place of the monoamides. The resulting water-in-oil emulsions exhibited the same properties of ready inversion and of foam prevention as did the emulsions in Examples I and II.

30 35 40 It will thus be seen that there is provided by this invention a new class of water-in-oil emulsions which are readily inverted by mere dilution and slight agitation. When such inversion occurs as the emulsions are added to aqueous stock, novel surface effects are obtained, similar to effects obtained by the use of unemulsified oils, but without the difficulties attending the use of unemulsified oils.

Having described our invention, what we claim as new and desire to secure by Letters Patent is:

45 50 55 1. A reversible emulsion of water in oil, the active emulsifying ingredient of which comprises chiefly a cationic surface active fatty amino compound, the fatty residue of which contains at least 10 carbon atoms and no hydrophilic groups, the amino compound being adjusted with acid to have a pH of about 6.0 or less in 2% aqueous solution.

2. A reversible emulsion of water in oil, the active emulsifying ingredient of which comprises chiefly the monoamide formed by reacting oleic acid and ethylene diamine, the monoamide being adjusted with acid to have a pH of about 6.0 or less in 2% aqueous solution.

60 65 70 3. A reversible emulsion of water in oil, the active emulsifying ingredient of which comprises chiefly the monoamide formed by reacting hydrogenated soyabean oil with ethanol ethylene diamine, the monoamide being adjusted with acid to have a pH of about 6.0 or less in 2% aqueous solution.

4. A reversible emulsion of water in oil, the active emulsifying ingredient of which comprises chiefly a fatty amine, the fatty residue of which contains at least 10 carbon atoms and no hydrophilic groups, the amine being adjusted with acid to have a pH of about 6.0 or less in 2% aqueous solution.

5. A reversible emulsion of water in oil, the active emulsifying ingredient of which comprises chiefly stearylamine, the stearylamine being adjusted with acid to have a pH of about 6.0 or less in 2% aqueous solution.

6. A reversible emulsion of water in oil, the active emulsifying ingredient of which comprises chiefly a cationic surface active fatty amino compound, the fatty residue of which contains at least 10 carbon atoms and no hydrophilic groups, the amino compound being adjusted by means of acetic acid to have a pH of about 6.0 or less in 2% aqueous solution.

7. A reversible emulsion of water in oil, the active emulsifying ingredient of which comprises chiefly a cationic surface active fatty amido-amine, the fatty residue of which contains at least 10 carbon atoms and no hydrophilic groups, the amido-amine being adjusted by means of acetic acid to have a pH of about 6.0 or less in 2% aqueous solution.

8. A reversible emulsion of water in oil, the active emulsifying ingredient of which comprises chiefly the monoamide formed by reacting oleic acid and ethylene diamine, the monoamide being adjusted by means of acetic acid to have a pH of about 6.0 or less in 2% aqueous solution.

9. A reversible emulsion of water in oil, the active emulsifying ingredient of which comprises chiefly a fatty amine, the fatty residue of which contains at least 10 carbon atoms and no hydrophilic groups, the amine being adjusted by means of acetic acid to have a pH of about 6.0 or less in 2% aqueous solution.

10. A defoaming agent comprising oil, water and an emulsifying agent which comprises chiefly a cationic surface active fatty amido-amine, the fatty residue of which contains at least 10 carbon atoms and no hydrophilic groups, the amido-amine being adjusted with acid to have a pH of about 6.0 or less in 2% aqueous solution.

11. Method of suppressing foam in aqueous process fluids which comprises adding thereto a reversible emulsion of water in oil, the active emulsifying ingredient of which comprises chiefly a cationic surface active fatty amino compound,

the fatty residue of which contains at least 10 carbon atoms and no hydrophilic groups, the amino compound being adjusted with acid to have a pH of about 6.0 or less in 2% aqueous solution.

5 12. Method of suppressing foam in aqueous process fluids which comprises adding thereto a reversible emulsion of water in oil, the active emulsifying ingredient of which comprises chiefly a cationic surface active fatty amido-amine, the fatty residue of which contains at least 10 carbon atoms and no hydrophilic groups, the amido-amine compound being adjusted with acid to have a pH of about 6.0 or less in 2% aqueous solution.

15 13. Method of suppressing foam in aqueous process fluids which comprises adding thereto a reversible emulsion of water in oil, the active emulsifying ingredient of which comprises chiefly the monoamide formed by reacting hydrogenated soyabean oil with ethanol ethylene diamine, the amide being adjusted with acid to have a pH of about 6.0 or less in 2% aqueous solution.

20 14. Method of suppressing foam in aqueous process fluids which comprises adding thereto a reversible emulsion of water in oil, the active emulsifying ingredient of which comprises chiefly a fatty amine, the fatty residue of which contains at least 10 carbon atoms and no hydrophilic groups, the amine being adjusted with acid to have a pH of about 6.0 or less in 2% aqueous solution.

25 15. Method of suppressing foam in aqueous process fluids which comprises adding thereto a reversible emulsion of water in oil, the active emulsifying ingredient of which comprises chiefly stearylamine, the stearylamine being adjusted with acid to have a pH of about 6.0 or less in 2% aqueous solution.

30 JAMES H. FRITZ.  
EDWIN A. ROBINSON.